

## UNITED STATES PATENT OFFICE

JOHN NEUMANN, OF CHICAGO, ILLINOIS

## FIBER BLEACHING

No Drawing.

Application filed March 29, 1929. Serial No. 351,127.

This invention relates to the bleaching of paper and other fiber pulps, and among other objects aims to reduce the time and cost of bleaching and to minimize loss of fiber and fiber strength. 5

The invention may best be disclosed by reference to an illustrative method embodying the invention and described in the following specification. The inventive method may advantageously be described as applied to the bleaching of kraft or sulphate pulp, since it is considered particularly difficult to bleach. 10

The kraft pulp is supplied in slush form of a consistency which may advantageously be about ten per cent. (10%). The process may be carried on in any appropriate apparatus provided with agitating means, means for heating the pulp both under and without pressure. It will be obvious, however, that the various steps of the process need not be carried out in a single piece of apparatus. While specially designed apparatus may be advantageously under certain conditions the process may be carried out in existing apparatus commonly employed in pulp treatment. 25

The unit proportions of treating substances used in the illustrative method will be based as is the usual practice, upon one ton of kraft pulp, air-dry weight. Into the apparatus above referred to is introduced an oxidizing agent, in this instance bleaching powder, in the amount of from fifty to one hundred (50 to 100) pounds. This ingredient is advantageously prepared in liquor form consisting of one (1) pound of bleaching powder per gallon of water. The quantity of bleaching powder used (between the limits above specified) depends upon the character of the water (whether it be hard or soft) and upon the character of the pulp, i. e. for example, whether it is a "hard cook" or "soft cook" pulp—the less oxidizing agent being used when the fibers are well opened up. In the apparatus the bleaching liquor is further diluted with a quantity of water which will bring the pulp, when added, to a consistency of from five to six per cent. (5% to 6%) of pulp. 40

By adding the pulp to the bleaching liquor (instead of vice versa) the burning of the

pulp, in spots, by the liquor is avoided. If the apparatus admits of it, the contents are agitated while the pulp is being added or while the bleaching liquor is added, if the sequence of the additions be reversed. 55

The pulp is then agitated for one hour at a temperature of from forty to eighty degrees Fahrenheit (40° to 80° F.), depending on the character of the pulp, the higher temperature stimulating action and being advantageous 60 for pulp in which the fibers are not well opened up.

The strength of the bleaching liquor used in the foregoing treatment is relatively weak but it bleaches the pulp to a yellow color. Its 65 action is not apparently primarily a bleaching one. It seems to attack the coloring matter and the fiber encrusting substances (with the possible exception of pitch) and thus prepares the pulp for the effective dissolving or removal by the next ensuing treatment, of those encrusting substances which have not already been eliminated. 70

In preparation for such treatment the bleaching liquor is withdrawn and the pulp 75 washed. It does no harm and possibly is advantageous to have a trace of the bleaching liquor remain in the pulp. This simplifies and shortens the washing of the pulp.

Into the same apparatus, assuming it to be 80 adapted for cooking under a low steam pressure (and from which the pulp may have been removed) an alkaline cooking liquor, in this instance comprising the following ingredients, is added: 85

10 pounds caustic potash.

100 pounds soda ash.

5 pounds sodium perborate

( $Na BO_3 \cdot 4 H_2O$ ).

Enough water is added to bring the consistency of the pulp, when added, to five or six per cent. (5% or 6%) of pulp. The above named ingredients are preferably added in the order named, i. e., with the perborate last. 90

The pulp is then added (again while the contents are agitated if that be possible) and the batch cooked and agitated for from thirty (30) minutes to one (1) hour (depending on the character of the pulp) at from two to five (2 to 5) pounds steam pressure. 95

100

This treatment apparently dissolves or removes the fiber encrusting substances without causing substantial loss of fiber or fiber strength. The perborate seems to cooperate to preserve the fiber strength, resulting in a quality and character of fiber particularly suitable for rayon and high grade alpha cellulose.

The liquor employed is then drained off and may be reclaimed and used again if restored to strength by addition of the chemicals exhausted. The pulp is then washed.

The pulp is now in condition where it will respond effectively to bleaching treatment.

I have found that satisfactory results may also be obtained if in the foregoing cooking treatment five (5) pounds of caustic potash and from forty to one hundred (40 to 100) pounds of sodium silicate (depending, as before, on character of fiber) be used in place of the caustic potash, soda ash and perborate,—other proportions and details of treatment remaining the same. Where appropriate, as with jack and southern pine and other highly resinous woods, such modified treatment commends itself because of the cheapness of the chemicals. If traces of silica remain in the pulp, the latter treatment would probably not be satisfactory if the pulp were to be used for rayon.

In the final bleaching treatment, a bleaching agent, in this case consisting of fifty (50) pounds of bleaching powder in liquor form (a concentration of one (1) pound of bleaching powder to a gallon of water), is introduced into an agitating vessel and water added to bring the consistency of the pulp, when added, to from five to six per cent. (5% to 6%). The washed pulp is then introduced and the contents agitated at a temperature of from forty to sixty degrees Fahrenheit (40° to 60° F.). A solution containing a reducing bleaching agent, in this instance three (3) pounds of oxalic acid and one (1) pound of common salt (NaCl), is also added but such addition can advantageously be deferred until the pulp and chlorine liquor have been agitated a short while. The total agitation and treatment should consume one (1) hour.

The interaction between the three chemicals in this treatment is not definitely understood but the effect of the treatment is to produce a dead white pulp. Treated with the chlorine liquor alone, the pulp, while bleached so that it can be termed bleached pulp and used commercially for many purposes as bleached pulp, is not dead white.

Apparently the oxalic acid acts only as a reducing or bleaching agent, but reacts with the chlorine (or perhaps there is a catalytic action) to stimulate the bleaching action and to carry it beyond the point which could be reached by successive treatments of the chlorine liquor and the oxalic acid and salt, of the strengths referred to. Apparently the

oxalic acid finally neutralizes the chlorine because the pulp requires little washing to bring it to a condition where there is no objectionable after effect, such as chlorine discoloration. The action of the salt is not fully understood,—apparently it reacts to temper the harsh characteristics of the oxalic acid, making it practically available in a bleaching process of this character.

After treatment for one hour and subsequent washing, the pulp is a dead white color and has substantially its original fiber strength. Although the entire process consumes a relatively short time bleaching has been accomplished without harsh treatment of the pulp and the loss of fiber and fiber strength has therefore been substantially minimized.

Obviously the invention is not limited to the precise chemical agents and other details of the illustrative method. With pulps which respond more readily to removal of encrusting substances or to bleaching, the length of treatment or strength of chemicals may be varied or even some of the chemicals omitted, or changed, depending upon the character and structure of the fiber, which characteristics are well known as regards most fiber yielding materials.

I claim:

1. The method of bleaching kraft pulp to a dead white color which is characterized by cooking the pulp to free the fibers from the encrusting substances and then treating the pulp with a bleaching agent containing 100 oxalic acid and sodium chloride.

2. The method of bleaching kraft pulp which is characterized by treating the pulp to free the fiber from encrusting matter and then bleaching the pulp by treatment with 105 chlorine liquor, oxalic acid, and sodium chloride.

3. The method of bleaching kraft pulp which is characterized by treating the pulp with chlorine liquor and then cooking it in an alkaline solution to remove the fiber encrusting substances, and then bleaching the pulp with chlorine liquor and oxalic acid in the presence of sodium chloride.

In testimony whereof, I have signed my 115 name to this specification.

JOHN NEUMANN.

120

125

130

**CERTIFICATE OF CORRECTION.**

**Patent No. 1,828,338.**

**Granted October 20, 1931, to**

**JOHN NEUMANN.**

**It is hereby certified that error appears in the printed specification of the above numbered patent requiring correction as follows: Page 2, line 58, after the word "acts" insert the word not; and that the said Letters Patent should be read with this correction therein that the same may conform to the record of the case in the Patent Office.**

**Signed and sealed this 15th day of December, A. D. 1931.**

**(Seal)**

**M. J. Moore,  
Acting Commissioner of Patents.**